

Jan. 23, 1962

E. GORIN

3,018,241

PRODUCTION OF HYDROGEN-RICH LIQUID FUELS FROM COAL

Filed Oct. 10, 1960

3 Sheets-Sheet 1



Fig. 1

INVENTOR.  
EVERETT GORIN

BY  
D. Leigh Fowler, Jr.  
ATTORNEY

Jan. 23, 1962

E. GORIN

3,018,241

## PRODUCTION OF HYDROGEN-RICH LIQUID FUELS FROM COAL

Filed Oct. 10, 1960

3 Sheets-Sheet 2



Tig 2

INVENTOR.  
*EVERETT GORIN*

BY  
D. Leigh Fowler, Jr.

**ATTORNEY**

Jan. 23, 1962

E. GORIN

3,018,241

## PRODUCTION OF HYDROGEN-RICH LIQUID FUELS FROM COAL

Filed Oct. 10, 1960

3 Sheets-Sheet 3



## 1

3,018,241

PRODUCTION OF HYDROGEN-RICH LIQUID  
FUELS FROM COALEverett Gorin, Pittsburgh, Pa., assignor to Consolidation  
Coal Company, Pittsburgh, Pa., a corporation of Penn-  
sylvania

Filed Oct. 10, 1960, Ser. No. 61,517

5 Claims. (Cl. 208—8)

The present invention relates to a method for converting coal to liquid hydrocarbons, and, more particularly, to the production of hydrogen-rich liquids suitable for use as feedstock in gasoline manufacturing operations.

This application is a continuation-in-part of my co-pending application Serial No. 802,768, filed March 30, 1959, now abandoned, which is a continuation-in-part of my application Serial No. 735,177, filed May 14, 1958, the latter application being abandoned on April 2, 1959, each of the above applications being assigned to the assignee of the present invention.

Of the many processes that have been proposed for conversion of coal to gasoline, those which involve only partial conversion of the carbon content of the coal to liquids are the most attractive economically. Any attempt to convert all the carbon of the coal to hydrocarbons must of necessity include the addition of large quantities of extrinsic hydrogen. Such addition is obviously expensive in view of the high cost of hydrogen. This is the major reason why there is no commercial coal-to-gasoline plant in this country today.

On the other hand, partial conversion of coal to liquid form offers attractive possibilities of making coal-to-gasoline plants a reality in the U.S. economy. The concept of partial conversion implies that optimum use is made of the hydrogen that is already present in the gross coal whereby it is preferentially distributed to a portion of the carbon content, leaving a hydrogen depleted residue. The generally accepted practical embodiment of partial conversion is low temperature carbonization, i.e. distillation of the coal in the temperature range of about 425° C. to 760° C. From such low temperature carbonization, a liquid, i.e. tar, is obtained which is hydrogen-rich in contrast to the solid residue, i.e. char which is hydrogen-depleted, as illustrated in the following Table I wherein the ultimate analyses in percent by weight are given on a moisture-free and ash-free basis (i.e. m.a.f.) for the tar and char respectively obtained by the carbonization of a Pittsburgh Seam coal at 496° C.

TABLE I

|   | Char | Tar  |
|---|------|------|
| H | 3.3  | 7.3  |
| C | 87.0 | 83.4 |
| O | 3.7  | 6.3  |
| N | 1.8  | 1.0  |
| S | 4.2  | 2.0  |

The liquid product of low temperature carbonization of coal, because of its hydrogen-rich character, has been hydrogenated commercially to make gasoline and other liquid fuels, for example, by the Germans. The coals employed, however, were relatively non-caking bituminous coals or the so-called brown coal. Such coals lend themselves readily to carbonization by any one of a number of different carbonization processes. In the case of highly caking coals, however, which are commonly found in this country, the potential yield of tar is difficult to achieve

## 2

at comparable cost because of the necessity for preventing agglomeration of the coal in the carbonization vessel. By way of illustration, the potential yield of tar from a highly caking coal of the Pittsburgh Seam, as determined by carbonization of the coal in the presence of sufficient inert diluent to prevent agglomeration, is in the range of 20 to 25 percent by weight of the m.a.f. coal. In a continuous process employing oxygen to "de-cake" the coal, the yield of tar drops to the range of 10 to 15 percent by weight of the m.a.f. coal. Thus, not only has the yield of the desired product been substantially reduced, but also the cost, because of the "de-caking" step, has increased.

The extraction of coal by means of solvents has been proposed as a kind of partial conversion of the coal. In some instances extraction has been accompanied by concurrent hydrogenation as by the use of extrinsic hydrogen, or by concurrent deposition of coke. The difficulty with such concurrent addition of hydrogen or concurrent rejection of carbon in the form of coke is that both are relatively non-selective, that is, not only is the extract subjected to such treatment, but so also is the coal residue. Thus, uncontrolled, indiscriminate, and inefficient redistribution of hydrogen is effected.

Coal extracts contain too many compounds of widely different molecular size to permit complete resolution of their component molecular species. However, it is sufficient for present purposes to examine the gross characteristics of the extracts in terms of molecular weight. Using benzene as a solvent, I have found that coal extracts may be separated readily into two fractions, a benzene-soluble and a benzene-insoluble fraction respectively. Surprisingly, the benzene-insoluble fraction has the following characteristics, set forth in Table II, regardless of the conditions, solvent used, or depth of extraction employed in the initial solvent extraction treatment.

TABLE II

|                           |                 |
|---------------------------|-----------------|
| Average molecular weight  | 1500            |
| Melting temperature range | 250° C.—350° C. |
| Hydrogen (wt. percent)    | 5.5 to 6.0      |

The entire ultimate analysis of the benzene-insolubles is similar to that of the feed coal except as to oxygen and sulfur. The benzene-solubles, on the other hand, vary in their characteristics depending on the conditions of extraction. In general, however, their molecular weight ranges from 300 to 1000, and their hydrogen content ranges from 6 to 8 percent by weight.

While the characteristics of the benzene-insoluble fraction of the extract, as set forth above, do not change significantly with increasing coal extraction, the amount of this portion in the extract increases materially with increasing coal extraction, in the absence of coking or hydrogen addition during the solvent extraction. This increase in amount of benzene-insolubles was observed in the case of all solvents tried, but at different rates of increase. I have further found that as the benzene-insoluble fraction of extract increases, the extract becomes correspondingly more difficult to hydrogenate, i.e., higher temperatures and pressures are required to convert substantially all the extract to hydrogen-enriched hydrocarbonaceous liquid.

The primary object of the present invention is to provide an improved process for converting bituminous coal, and particularly a highly caking bituminous coal, to a hydrogen-enriched liquid suitable as feedstock for gasoline manufacturing operations.

Another object of this invention is to provide a com-

bination process for converting coal to a gasoline feedstock which process combines, to best advantage in selective fashion, low temperature carbonization, solvent extraction, coking of liquids, and hydrogenation.

A further object of this invention is to provide a process for producing a hydrogen-enriched liquid suitable as a gasoline feedstock, which process comprises hydrogenating under optimum conditions a hydrogen-enriched liquid product derived from coal by a novel combination of coal processing steps.

A still further object of the present invention is to provide a process for converting coal to a hydrogen-enriched liquid suitable as a gasoline feedstock wherein the necessary hydrogen is substantially entirely derived from the coal feedstock.

In accordance with my invention, bituminous coal is partially dissolved in a hydrocarbonaceous solvent at elevated temperatures under substantially non-coking conditions. The amount of coal dissolved under the extraction conditions is limited to less than 80 percent by weight of the m.a.f. coal (m.a.f. signifies moisture-free and ash-free). A part of the extract consisting predominantly of benzene-insoluble material is separated from the extract. This benzene-insoluble fraction is coked alone or in combination with the undissolved portion of the coal, i.e. residue, to yield a benzene-soluble product. All or selected fractions of the liquid products including the remainder of the extract are combined and hydrogenated to yield a high quality gasoline feedstock.

In the preferred embodiment of my invention, the solvent extraction treatment is controlled to yield an extract, under the extraction conditions, which amounts to less than 60 percent by weight of the m.a.f. coal. I have found it desirable in certain cases to subject the coal to solvent extraction conditions such that between 60 and 80 percent by weight of the m.a.f. coal is dissolved. However, in such cases it is necessary to separate sufficient benzene-insoluble material from the extract so that less than 65 percent by weight of the m.a.f. coal is recovered as the benzene-soluble rich fraction, as will be more fully explained hereinafter.

For a better and more complete understanding of my invention, its objects and advantages, reference should be had to the following detailed description and to the accompanying drawings in which:

FIGURE 1 is a graph showing the relationship of hydrogen transferred from solvent to coal to the depth of extraction;

FIGURE 2 is a schematic flow sheet of the preferred embodiment of my invention; and

FIGURE 3 is a schematic flow sheet of an alternative embodiment of my invention.

#### *Preferred embodiment*

Referring to FIGURE 2 of the drawings, comminuted coal is introduced into a stirred solvent extraction zone 10 concurrently with 0.5 to 4.0 parts by weight of a solvent. The extraction zone 10 is adapted to confine the coal and the solvent for a residence period from about five minutes to four hours at elevated pressures and temperatures. The residence period and temperatures are determined by the specific solvent and the desired depth of coal extraction. The pressure is that required to maintain the solvent as a liquid at the selected temperature, generally in the range of 1 p.s.i.g. to 6500 p.s.i.g.

Suitable solvents for the coal in the extraction step are those which are predominantly polycyclic hydrocarbons, preferably partially or completely hydrogenated aromatics, including naphthenic hydrocarbons, which are liquid under the temperature and pressure of extraction. Mixtures of these hydrocarbons are generally employed, and are derived from intermediate or final steps of the process of this invention. Those hydrocarbons

or mixtures thereof boiling between about 260° C. and 425° C. are preferred. Examples of suitable solvents are tetralin, decalin, biphenyl, methylnaphthalene, and dimethylnaphthalene. Other types of coal solvent may be added to the above-mentioned types for special reasons, but the resulting mixture should be predominantly of the types mentioned, i.e. should constitute more than 50 percent by weight of the solvent used. Examples of additive solvents are the phenolic compounds, such as phenol, cresols and xylenols.

As stated above, the coal is comminuted, and preferably, but not necessarily, of a fluidizable size, for example —14 mesh Tyler Standard screen. Up to about 25 percent depth of extraction, the coal particles retain substantially their original size; beyond 25 percent extraction, the particles undergo degradation.

The coal and the solvent are maintained in intimate contact within the extraction zone 10 until the solvent has dissolved the desired amount of coal, i.e. up to 80 percent by weight of the m.a.f. coal. At least 10 percent by weight of the m.a.f. coal should be dissolved since the extract below 10 percent is essentially benzene-soluble material and therefore does not require the use of my process. To dissolve above about 40 percent of the m.a.f. coal, it is normally necessary that hydrogen be added to the coal. This is usually accomplished by employing hydrogen-transferring solvents such as tetralin or mixtures of hydrocarbons derived from intermediate or final steps of the process. I have found that as one increases the depth of extraction, the transfer of hydrogen increases rapidly (as is demonstrated by reference to FIGURE 1 of the drawings) such that if the depth of extraction exceeds 80 percent, the over-all process becomes economically prohibitive in terms of the cost of the hydrogen required. Specifically, at high depths of extraction, the hydrogen does not react exclusively with the new-forming extract, but instead produces an increasing amount of gas which is of little value as compared to the extract. In FIGURE 1 the hydrogen transferred (wt. percent of m.a.f. coal) to the extract from the solvent is plotted against depth of extraction.

As previously stated, as one increases the depth of extraction, each additional increment of extract contains a higher proportion of benzene-insoluble material. Thus, the deeper one extracts, the greater the amount of benzene-insoluble material that must be separated from the extract. In order to minimize the amount of benzene-insolubles that must be separated, I prefer to conduct the solvent extraction under conditions to yield an extract amounting to less than 60 percent by weight of the m.a.f. coal.

The temperature of the extraction zone should be an elevated temperature between about 100° C. and 500° C., but in no event high enough to cause appreciable coke formation. In some instances it may be desirable to conduct the extraction in stages at successively higher temperatures until the desired depth of extraction is attained. Instead of a batch system, a continuous countercurrent system may be employed. The particular system used is not material to the practice of my invention.

Following extraction, the mixture of solvent, extract, and residue is conducted rapidly, so as to avoid cooling of the mixture, through a conduit 12 to a stirred separation zone 14. The primary function of this zone is to separate the extract into a benzene-insoluble rich fraction and a benzene-soluble rich fraction. This separation may be accomplished by the addition to the separation zone 14 of a paraffinic solvent, e.g. hexane, in a volume ratio of the paraffinic solvent to the extraction solvent between 0.1 and 1.0. Alternatively, the temperature of the separation zone may be lowered below the temperature employed in the solvent extraction zone. Depending upon the coal solvent employed, the temperature of extraction, and the depth of extraction, the

act of cooling to low temperature may precipitate most of the benzene-insoluble rich fraction, thereby dispensing with the necessity of adding the precipitating paraffinic solvent. If a paraffinic solvent is used, I have found that the solvent is useful as an aid to the subsequent separation of the solids from the liquid. It is important in any event to have determined in advance the amount of benzene-insolubles in the extract so that the precipitation of the desired amount of the extract can be controlled. The larger the amount of benzene-insolubles in the extract, the larger is the amount of precipitating solvent that must be added, or the greater is the difference in temperature between the extraction zone and the separation zone that must be maintained.

From the separation zone 14 a mixture of liquid and solids is discharged through a conduit 16 to a conventional type filtration zone 18, or if desired a centrifuge. The solids are therein separated from the liquid. The liquid phase, consisting of a solution of the benzene-soluble rich fraction of the extract and solvents, i.e., the paraffinic solvent, if used, and the extraction solvent, is conducted through a conduit 20, to a fractionation zone 22 wherein the extraction solvent is recovered and recycled through a conduit 24 to the extraction zone 10; and the precipitating solvent, if used, is recovered and returned through a conduit 26 to the separation zone 14.

The benzene-soluble rich fraction of the extract is separately recovered and conducted through a conduit 28 to a hydrogenation zone 30, the operation of which will be hereinafter described. If desired, some or all of the extraction solvent, instead of being recycled to the extraction zone 10, may be used as a diluent for the benzene-soluble rich fraction in its passage through the hydrogenation zone.

As pointed out earlier, it may be desirable to dissolve up to 80 percent by weight of m.a.f. coal. Depending on the coal employed, the solvent used, as well as other extraction conditions, there may be sufficient benzene-soluble material present in the incremental extracts beyond 60 percent to justify its recovery. However, to recover this additional benzene-soluble material requires substantial separation of the incremental benzene-insoluble material. I have found it to be necessary to separate at least sufficient benzene-insoluble material to ensure recovery of less than 65 percent of the m.a.f. coal as the benzene-soluble rich fraction.

The solids from the filtration zone 18, i.e. the residue and the precipitated benzene-insoluble rich fraction of the extract, are discharged into a conduit 32 where they are picked up by a stream of recycle gas, air, or steam entering through a conduit 34 and are carried into a carbonization zone 36. It should be noted at this point that, if desired, the residue from the extraction zone 10 may be separated from the extract as by filtration prior to separating the extract into the benzene-soluble and benzene-insoluble rich fractions. In such a case the residue is sent directly to the carbonization zone 36, and the extract is then introduced into the separation zone 14. The benzene-insoluble rich fraction may then be coked separately or introduced into the carbonization zone 36. The carbonization zone 36 may be any one of the well-known systems for carbonizing carbonaceous solids at low temperatures, i.e., 425° C. to 760° C. For example, a bed of solids may be maintained in the zone in a fluidized state by means of the above-mentioned carrier gas. The temperature of the carbonization zone may be maintained by any suitable means, for example, by preheating the carrier gas to the appropriate high temperature. I prefer, however, to burn a portion of the carbonized residue, i.e. char, produced in the carbonization zone 36 to supply the necessary heat. This is accomplished by withdrawing char from the carbonization zone 36 through a conduit 38, and conveying the withdrawn char by means of an inert gas such as recycle gas entering through a conduit 40 into a char devolatilization zone 42. The char is pref-

erably maintained in a fluidized state in this zone at a temperature between about 645° C. and 945° C. The devolatilization temperature must be higher than any processing temperature to which the solids have been previously exposed. The volatile content of the solids will be driven off as a hydrogen-rich gas which can be recovered through a conduit 44. A typical composition of such gas produced by simply heating char (derived by carbonization at 496° C.) at 870° C. is in percent by volume as follows: H<sub>2</sub>—72.0; H<sub>2</sub>S—0.75; CO<sub>2</sub>—0.81; CO—13.19; CH<sub>4</sub>—12.15; and N<sub>2</sub>—1.1. Devolatilization of char to produce hydrogen-rich gas is further described and claimed in my copending application, Serial No. 144,423, filed October 11, 1961, which is assigned to the assignee of the present application. A portion of the devolatilized char is withdrawn from the devolatilization zone 42 through a conduit 46; picked up by air entering through a conduit 48, and lifted through a combustion leg 50. The temperature of the char as a result of the combustion is raised to that sufficient to maintain the temperature in the devolatilization zone 42 when returned through a cyclone separator 52 and a conduit 54 to that zone. Flue gas is removed from the cyclone separator 52 through a conduit 56. Hot char from the devolatilization zone 42 is transferred by a conduit 58 back to the carbonization zone 36 by means of recycle gas from the conduit 40. Net char produced in the carbonization zone is discharged through a conduit 60. The hydrogen-rich gas from the char devolatilization zone 42 is conducted via the conduit 44 to a conversion zone 62 where substantially pure hydrogen is produced by techniques well known in the art. The resulting hydrogen is conveyed through a conduit 64 to a compressor 66 which compresses the hydrogen to the desired pressure. The compressed hydrogen is conducted to the hydrogenation zone 30 through a conduit 68.

Returning to the carbonization zone 36, the effluent tar vapors are circulated through cyclone separators 70 and 72, which return finely divided solids to the carbonization zone 36. The tar vapors are conducted through a conduit 74 to a condenser 76 where non-condensable gas is discharged through a conduit 78. The gas may be used for manufacture of hydrogen by known methods such as steam reforming or may be used as plant fuel. The tar is carried through a conduit 80 to a fractionation zone 82 in which a liquid fraction boiling below 325° C. and a liquid fraction boiling above 325° C. are recovered. The fraction boiling below 325° C. is discharged through a conduit 84 which leads to the conduit 24 emptying into the extraction zone 10. If desired, however, a portion of the low boiling fraction may be recovered through a conduit 86 and thence introduced into a gasoline refining plant. The fraction boiling above 325° C., after suitable treatment (not shown) to remove any solids, if present, is discharged into a conduit 88 which conveys the fraction to the conduit 28 wherein it is commingled with the benzene-soluble rich fraction.

The mixture of the benzene-soluble rich fraction and the tar in conduit 28 contains asphaltic materials or asphaltenes which have an average molecular weight between about 700 and 1000. In some instances it may be desirable to reduce the asphaltene content. Accordingly, a deasphalting zone 90 may be interposed in the conduit 28 for precipitating at least a portion of the asphaltenes. The deasphalting is accomplished by well-known methods employed in petroleum technology such as the addition of propane, pentane, or hexane. The precipitated asphaltenes, preferably diluted with a fluxing oil such as a portion of a coker distillate, are conducted through a conduit 92 to a preheater 94 and thence into a coking zone 96 adapted in conventional fashion to coke the asphaltenes at a temperature between about 426° C. and 760° C. Ash-free coke is discharged through a conduit 98. The coker distillate is removed through a conduit 100 and condensed in a condenser 102, from which non-condensable

gases are discharged through a conduit 104. The condensate is carried by a conduit 106 back to the conduit 28 leading to the hydrogenation zone 30. An added advantage of the deasphalting step is the removal of any residual carbonaceous solids carried over into the benzene-soluble rich fraction of the extract or the tar as the case may be.

Preferably, however, the mixture of benzene-soluble rich extract and the tar from the fractionation zone 82, recovered via the conduit 88, is introduced directly into the hydrogenation zone 30.

In the hydrogenation zone 30, the extract and tar are contacted with hydrogen, preferably in the presence of a hydrogenation catalyst. As previously mentioned, hydrogen is introduced into the hydrogenation zone 30 via the conduit 68; however, if required, additional hydrogen may be introduced into the system through a conduit 108 at the compressor 66. Hydrogenation of the extract and tar can be conducted at pressures of 1000 p.s.i.g. to 10,000 p.s.i.g., preferably about 2000 p.s.i.g. to 3500 p.s.i.g., a range well below that normally required for direct hydrogenation of coal. The hydrogenation temperature range is about 400° C. to 600° C., preferably about 410° C. to 455° C. The hydrogenation catalyst should be sulfur-resistant, e.g., molybdenum or tungsten oxides or sulfides impregnated on a refractory support to permit catalyst regeneration. The support usually will be an alumina-rich material such as pure gamma alumina or alumina composited with other oxides such as silica. Other metals such as nickel or cobalt may be added as catalyst promoters.

The products of hydrogenation are discharged from the hydrogenation zone 30 through a conduit 110, cooled, and passed into a separator 112. Hydrogen-rich gas is separated from the products and recycled through a conduit 114 to the hydrogenation zone 30. The remaining products in the separator 112 are depressurized and then passed via a conduit 116 into a low pressure separator 118. From the low pressure separator 118 the liquid product is carried through a conduit 120 to a fractionation zone 122, while the gaseous product is withdrawn from the separator 118 via a conduit 124. The liquid product is fractionated in the fractionation zone 122 into any desired fractions. A preferred separation is to fractionate the liquid hydrogenation product into a fraction boiling above 360° C. and a fraction boiling below 360° C. The latter fraction is passed through a conduit 126 to further refining and hydrogenation operations for conversion to gasoline in conventional fashion. The former fraction is passed through a conduit 128 and may be reintroduced into the hydrogenation zone 30 or into the coking zone 96. If desired, portions of both fractions may be introduced into the solvent extraction zone 10, as a portion of the solvent therein.

#### EXAMPLE I

The embodiment of the present invention shown in FIGURE 2 and described above is illustrated by the following example pertaining to Pittsburgh Seam caking bituminous coal.

The coal was subjected to an extraction in a closed vessel with decalin as a solvent at a temperature of 348° C. for one hour. Based on 100 pounds of m.a.f. coal, 220 pounds of decalin were employed as solvent. The ultimate analysis of the starting coal and the solvent-free extract is as follows:

|   | MAF Coal,<br>Weight<br>Percent | Extract,<br>Weight<br>Percent |
|---|--------------------------------|-------------------------------|
| H | 5.74                           | 6.45                          |
| C | 82.26                          | 83.51                         |
| N | 1.31                           | 1.23                          |
| O | 8.13                           | 6.81                          |
| S | 2.56                           | 2.00                          |

The yields of extraction products, based on 100 pounds of m.a.f. coal, are as follows:

|                        | Weight of product<br>(pounds) |
|------------------------|-------------------------------|
| Hydrogen sulfide       | 0.1                           |
| Gas                    | 1.0                           |
| Liquor                 | 1.0                           |
| Extract                | 23.0                          |
| Solid residue (m.a.f.) | 74.9                          |

The addition of 50 pounds of hexane to the extract solution precipitated 6.2 pounds of extract of which about 70 percent by weight was determined to be benzene insoluble. The remainder of the extract contained about 85 percent by weight of benzene-soluble material. The precipitated extract and solid residue were carbonized at 510° C., yielding 58.5 pounds of char and 12.6 pounds of tar including the light oil fraction. The total yield of liquid was thus 29.2 pounds.

In the description of the preferred embodiment, the deasphalting step (see 90 of FIGURE 2) and the coking of the precipitated asphaltenes (see 96 of FIGURE 2) may be eliminated and, instead, the +360° C. oil from the hydrogenation zone 30 be recycled through that zone. Or as a still further option, the deasphalting step may be eliminated with the +360° C. oil from the hydrogenation zone 30 going to the coker 96. In order to compare these three optional modes of treatment of the hydrogenation feedstock, the above-mentioned liquid yield of 29.2 pounds was divided into three aliquot parts which were respectively subjected to the three optional treatments.

The first aliquot part, hereinafter called Aliquot A, was treated in accordance with the steps shown in FIGURE 2, namely, as follows, with the understanding that the yields are reported on the basis of a starting feedstock of 29.2 pounds, that is, the actual yield is multiplied by three. To Aliquot A was added 20 pounds of hexane per 100 pounds of Aliquot A. The resulting precipitate comprising principally asphaltenic material amounted to 4.6 pounds. The latter was coked in a conventional delayed coking system at 470° C., yielding 2.7 pounds of ash-free coke and 1.4 pounds of coker distillate. The latter was combined with the non-precipitated portion of the extract from the deasphalting step, making a total of 26.0 pounds, which was then hydrogenated in a fixed bed catalyst system. The catalyst was cobalt molybdate on alumina (15% MoO<sub>3</sub>—3% CoO—82% Al<sub>2</sub>O<sub>3</sub>); the temperature was 440° C.—454° C., and the pressure 3500 p.s.i.g. The liquid hourly space velocity was about 1.0 pound of total feed per pound of catalyst per hour. The hydrogenated products were fractionated and the —360° C. distillate recovered as gasoline feedstock. The +360° C. fraction amounting to 10.4 pounds was recycled through the hydrogenation zone 30. The amount of H<sub>2</sub> consumed was 1.22 pounds.

The second aliquot part, hereinafter designated Aliquot B, was simply sent directly to the hydrogenation zone without any deasphalting or coking treatments. The same hydrogenation conditions were employed as used for Aliquot A. The hydrogenated products likewise were fractionated yielding 25.8 pounds of —360° C. gasoline feedstock and some +360° C. oil which was recycled through the hydrogenation zone. The amount of H<sub>2</sub> consumed was 1.46 pounds.

The third aliquot part, hereinafter designated as Aliquot C, like Aliquot B, was sent directly to the hydrogenation zone and hydrogenated under the same conditions as were the other aliquot parts. The resulting hydrogenated products were similarly fractionated into a —360° C. fraction (23.5 pounds) and a +360° C. fraction (10.6 pounds). The latter was coked in the above-mentioned delayed coking system at 468° C., yielding 1.8 pounds of ash-free coke and 8.1 pounds of coker distillate which was mixed with Aliquot C before entering the hydrogenation zone.

The results of the above-described treatments may be summarized as follows:

TABLE III

Composition of the several feed materials

|                                                           | H    | C    | N   | O   | S   |
|-----------------------------------------------------------|------|------|-----|-----|-----|
| Raw Extract                                               | 6.45 | 83.5 | 1.2 | 6.8 | 2.0 |
| Extract with Benzene Insolubles Removed                   | 6.69 | 83.1 | 1.0 | 7.2 | 2.1 |
| Tar from Low Temperature Carbonization                    | 7.60 | 83.3 | 1.0 | 6.5 | 1.6 |
| Coker Distillate Aliquot A                                | 7.31 | 86.1 | 1.0 | 4.2 | 1.4 |
| Average Recycle Oil to Hydrogenation Zone                 | 9.07 | 89.9 | 0.4 | 0.5 | 0.1 |
| Total Feed to Hydrogenation Zone (Excluding Recycle Oil): |      |      |     |     |     |
| Aliquot A                                                 | 7.24 | 82.9 | 0.9 | 7.0 | 2.0 |
| Aliquots B and C                                          | 7.08 | 83.1 | 1.0 | 6.9 | 1.9 |

TABLE IV

Feed composition to hydrogenation zone and total yields

|                                                                  | Aliquot A Case | Aliquot B Case | Aliquot C Case |
|------------------------------------------------------------------|----------------|----------------|----------------|
| Wt. Percent of Feed to Hydrogenation Zone:                       |                |                |                |
| Extract and Tar                                                  | 71.5           | 66.7           | 78.3           |
| Recycle Oil                                                      | 28.5           | 33.3           | 21.7           |
| Yield Wt. Percent of MAF Coal:                                   |                |                |                |
| -360° C. Distillate                                              | 23.2           | 25.8           | 23.5           |
| Gas                                                              | 1.7            | 1.8            | 2.2            |
| Liquor                                                           | 1.9            | 2.1            | 2.1            |
| H <sub>2</sub> S                                                 | 0.5            | 0.6            | 0.5            |
| Ash-free Coke                                                    | 2.7            | 0.0            | 1.8            |
| H <sub>2</sub> Consumption                                       | 1.22           | 1.46           | 1.34           |
| Lbs. H <sub>2</sub> Consumed per 100 lbs. of -360° C. Distillate | 5.25           | 5.66           | 5.69           |

## EXAMPLE 2

Pittsburgh Seam coal was subjected to a solvent extraction in a closed vessel with tetralin at a temperature of 380° C. for 52 minutes. Based on 100 pounds of m.a.f. coal, 200 pounds of tetralin were employed. The yields of extraction products based on 100 pounds of m.a.f. coal are as follows:

|                      | Weight of product (pounds) |
|----------------------|----------------------------|
| Extract              | 68.3                       |
| Residue (m.a.f.)     | 23.5                       |
| Gas+liquor+light oil | 8.2                        |
|                      | 100.0                      |

The extract and residue mixture was then filtered at about 205° C., and as a result of the drop in temperature, 8.3 pounds of the extract precipitated onto the residue. The remaining extract, i.e. the benzene-soluble rich fraction, amounting to 60.0 pounds, was recovered from the filtration zone and catalytically hydrogenated, while the solids, i.e. the residue and the precipitated benzene-insoluble rich portion of the extract, were withdrawn from the filtration zone and then introduced into a carbonization zone.

The analysis of the precipitated extract and the benzene-soluble rich fraction is as follows:

|                    | Precipitated Extract, Percent | Benzene-Soluble Fraction, Percent |
|--------------------|-------------------------------|-----------------------------------|
| Benzene-Solubles   | 3.1                           | 61.2                              |
| Benzene-Insolubles | 96.9                          | 38.8                              |
|                    | 100.0                         | 100.0                             |

## Alternative embodiment

An alternative embodiment of the present invention is illustrated in FIGURE 3 of the drawings. The chief distinction between the preferred embodiment and the alter-

native embodiment lies in the treatment of the extract, as the following description will show.

Referring now to FIGURE 3, in order to avoid unnecessary duplication of description, those parts of the alternative embodiment operating the same as corresponding parts of the preferred embodiment have been designated by the same numerals. The mixture of extract and residue produced in the extraction zone 10 is conveyed through a conduit 11 to the filtration zone 18 where the extract is separated from the residue. The latter is conveyed through a conduit 13 to a drying zone 15 wherein steam entering through a conduit 17 is employed to strip any retained solvent from the residue. The effluent stream from the dryer is passed through a conduit 19 to a pair of cyclone separators 21 which separate the vapors from the solids. The solids drop into a conduit 23 where they are picked up by recycle gas and introduced into the carbonization zone 36. The operation of this zone, together with the char devolatilization zone 42 and the char combustion leg 50, is the same as that described in connection with the preferred embodiment.

The extract is conducted through a conduit 25 to a flash tower 27 where at least some of the solvent is flashed off through a conduit 29. The solvent vapors are commingled with solvent vapors from the residue dryer 15 in a conduit 31 which carries them to a condenser 33. Any non-condensable gas is discharged through a conduit 35 while the condensed solvent is returned to the extraction zone 10, via a conduit 37.

The extract is conveyed from the flash tower 27 through a conduit 39 to a preheater 41 which serves to raise the temperature of the extract to about 426° C. to 468° C. The preheated extract is passed through a mild prehydrogenation zone 43 which serves to add about 0.5 to 2.0 pounds of hydrogen per 100 pounds of feed. The operating conditions are as follows:

Temperature: 425° C. to 470° C., preferred 440° C. to 455° C.

Pressure: 500-2500 p.s.i.g.

Residence time: 5-60 minutes, preferred 10-30 minutes.

Hydrogen input to the prehydrogenator 43 may be by means of hydrogen transfer from hydrogenated middle oil derived from the final step of the present process. Free hydrogen gas may also be added to aid hydrogenation. The operation is conducted substantially non-catalytically, or with relatively small amounts of "homogeneous" catalysts, i.e., .05 to 1.0 weight percent of a hydrogen halide or its corresponding ammonium salt, i.e., NH<sub>4</sub>Cl, NH<sub>4</sub>Br, or NH<sub>4</sub>I. Inexpensive catalysts such as red mud may also be used if desired. The hydrogenated middle oil is used in amounts between 1 and 3 parts per part of extract, preferably mixed with solvent from flash tower 27. Mild prehydrogenation of extract is further described and claimed in my copending application, Serial No. 144,428, filed October 11, 1961, which is assigned to the assignee of the present application.

The mildly hydrogenated extract is discharged through a conduit 45 into a fractionation zone 47 which serves to separate the extract into a +325° C. and a -325° C. fraction. The latter fraction is sent directly through a conduit 49 to the hydrogenation zone 30. The +325° C. fraction is conveyed through a conduit 51 into a conduit 53 to a preheater 55 and thence through a conduit 57 to a coking zone 59 operating at 425° C. to 760° C. Ash-free coke is discharged through conduit 61. Coker distillate is withdrawn from the coking zone 59 via a conduit 63 and is commingled with the tar vapors withdrawn from the carbonizer 36 via a conduit 65. The mixture is then introduced into a fractionator 67. A -300° C. fraction is recovered through a conduit 69 for further refining, if desired, to yield chemicals and low boiling solvents. A 300° C. to 425° C. fraction is sent through a conduit 71 to a preheater 73 and thence

via conduits 75 and 49 into the hydrogenation zone 30. A +425° C. fraction is recycled through a conduit 77 to the coking zone 59. The hydrogenated products from the hydrogenation zone 30 are conveyed through a conduit 79 to the fractionator 122 and therein separated into gasoline feedstock recovered through the conduit 126 and a make-up solvent stream recovered through the conduit 128.

According to the provisions of the patent statutes, I have explained the principle, preferred construction, and mode of operation of my invention and have illustrated and described what I now consider to represent its best embodiment. However, I desire to have it understood that, within the scope of the appended claims, the invention may be practiced otherwise than as specifically illustrated and described.

I claim:

1. A combination process for the production of hydrogen-enriched liquid fuels from coal which comprises subjecting the coal to solvent extraction under conditions to dissolve less than 80 percent by weight of the m.a.f. coal, whereby an extract containing both benzene-soluble and benzene-insoluble material is obtained, separating from the products of extraction undissolved coal residue and a first and a second extract fraction, said first fraction being richer in benzene-insoluble material than said second fraction and said second fraction amounting to less than 65 percent by weight of the m.a.f. coal, subjecting said residue and said first extract fraction to carbonization under conditions yielding liquid distillates, combining at least a portion of said second extract fraction with at least a portion of said distillates, subjecting the resulting mixture to hydrogenation under conditions to yield a gasoline feedstock, and recovering said gasoline feedstock.

2. A combination process for the production and recovery of liquid hydrocarbons from coal which comprises subjecting the coal to solvent extraction in a solvent containing predominantly hydrocarbons selected from the class consisting of polycyclic aromatic and polycyclic hydrogenated aromatic hydrocarbons and mixtures thereof under conditions to yield an extract amounting to less than 60 percent by weight of the m.a.f. coal, adding a paraffinic solvent to the extraction mixture of solids and solution in sufficient quantity to precipitate a portion of the extract which contains predominantly benzene-insoluble material, separating the extract solution from the coal residue and precipitate, adding a deasphalting solvent to the separated extract in sufficient quantity to precipitate at least a portion of the asphaltenes, carbonizing coal residue, the precipitated benzene-insoluble portion and the asphaltene portion at 425° C. to 760° C., subjecting at least a portion of the liquid products from the aforesaid process steps to hydrogenation and recovering the resulting hydrogenated products.

3. A combination process for the production of hydrogen-enriched liquid fuels from coal which comprises subjecting the coal to solvent extraction under conditions to yield an extract amounting to less than 60 percent by weight of the m.a.f. coal and containing both benzene-soluble and benzene-insoluble material, separating from the products of extraction undissolved coal residue and a first and a second extract fraction, said first fraction being richer in benzene-insoluble material than said second fraction, subjecting said residue and said first extract fraction to carbonization under conditions yielding liquid distillates, combining at least a portion of said second extract fraction with at least a portion of said distillates, subjecting the resulting mixture to hydrogenation under conditions to yield a gasoline feedstock, and recovering said gasoline feedstock.

4. A combination process for the production of hydrogen-enriched liquid fuels from coal which comprises subjecting the coal to solvent extraction under conditions to yield an extract amounting to less than 60 percent by weight of the m.a.f. coal and containing both benzene-soluble and benzene-insoluble material, separating from the products of extraction undissolved coal residue and a first and a second extract fraction, said first fraction being richer in benzene-insoluble material than said second fraction, further separating from said second extract fraction a third and a fourth extract fraction, the third fraction being richer in asphaltenes than the fourth fraction, subjecting said residue, said first extract fraction, and said third extract fraction to carbonization under conditions yielding liquid distillates, combining at least a portion of said fourth fraction with at least a portion of said liquid distillates, subjecting the resulting mixture to hydrogenation under conditions to yield a gasoline feedstock, and recovering said gasoline feedstock.

5. A combination process for the production of hydrogen-enriched liquid fuels from coal which comprises subjecting the coal to solvent extraction under conditions to dissolve between 60 and 80 percent by weight of the m.a.f. coal, whereby an extract containing both benzene-soluble and benzene-insoluble material is obtained, separating from the products of extraction undissolved coal residue and a first and a second extract fraction, said first fraction being richer in benzene-insoluble material than said second fraction, said second fraction comprising less than 65 percent by weight of the m.a.f. coal, subjecting said residue and said first extract fraction to carbonization under conditions yielding liquid distillates, combining at least a portion of said second extract fraction with at least a portion of said distillates, subjecting the resulting mixture to hydrogenation under conditions to yield a gasoline feedstock, and recovering said gasoline feedstock.

No references cited.